

No. 763,260.

PATENTED JUNE 21, 1904.

A. E. CATTERMOLE.

## SEPARATION OF THE METALLIC CONSTITUENTS OF ORES FROM GANGUE.

APPLICATION FILED JAN. 2, 1904

NO MODEL.



Wortweiss  
Franklin  
Jan R Adams

W. H. F. Inventor:  
William E. Rattner, Jr.

By Knight & Coz  
Attorneys

## UNITED STATES PATENT OFFICE.

ARTHUR EDWARD CATTERMOLE, OF HIGHGATE, LONDON, ENGLAND.

## SEPARATION OF THE METALLIC CONSTITUENTS OF ORES FROM GANGUE.

## SPECIFICATION forming part of Letters Patent No. 763,260, dated June 21, 1904.

Original application filed September 28, 1903, Serial No. 174,947. Divided and this application filed January 2, 1904. Serial No. 187,599. (No specimens.)

*To all whom it may concern:*

Be it known that I, ARTHUR EDWARD CATTERMOLE, a subject of the King of England, residing at Highgate, London, England, have 5 invented certain new and useful Improvements in the Separation of the Metallic Constituents of Ores from Gangue, of which the following is a specification.

This application is a division of my application filed September 28, 1903, Serial No. 174,947.

The present invention relates to improvements in the separation of the metalliferous constituents of ores and the like from gangue 15 by means of the selective action of oils and certain tar products or similar compounds (all hereinafter referred to as "oil") on metallic or metalliferous matter.

The invention depends upon the application 20 of the following facts: First, when a mixture of powdered metalliferous matter and gangue is treated with oil suspended in water—that is to say, in emulsion—the oil has a more or less selective action and will 25 coat the particles of metalliferous matter in preference to the particles of gangue, while the particles of gangue will be wetted by the water; second, if the water be made alkaline and an emulsifying agent, such as soap, be 30 present, the selective action of the oil will be rendered more marked and decisive; third, if the proportion of oil is kept within reasonably low limits (differing in different cases, according to the nature of the mineral to be 35 treated and the consistency and nature of the oil) and if the mixture of water, oil, metalliferous particles, and gangue be thoroughly agitated, the metalliferous particles which have become coated with oil will adhere together 40 and form granules, which granules, partly by reason of gravity or partly on account of their bulk as compared with the individual grains of gangue, will offer ready means for separation in an upcurrent-separator, a jig, or other similar appliance. This 45 action is facilitated if the oil before addition to the liquor is brought into the condition of an emulsion in water containing a small percentage of free soap.

In some cases the pulp may contain mineral 50 acid. Alkali must then be added in sufficient quantity to neutralize the acid and to leave some alkaline soap undecomposed—that is, free.

These facts are utilized for the purpose of 55 separating the metalliferous constituents from the gangue of the ore in the following manner: In a suitable apparatus, an example of which will be hereinafter described, the ground or pulped ore is caused to be violently 60 agitated, as by a revolving stirrer, in a mixture of water and oil, the liquor containing an alkaline emulsifying agent. As the agitation proceeds the particles of metalliferous matter 65 agglomerate together and may be observed in the form of granules, the size of which will depend, among other things, upon the percentage of oil used. This granulation of the metalliferous constituents of the ore affords 70 the means by which at a later stage of the process it is possible to separate the metalliferous material from the gangue, as will be hereinafter particularly described. In practice a continuous process is used—that is to say, water, ground ore, or pulp and oil, preferably 75 emulsified, are continuously fed into a series of vessels and the products of the agitation are continuously fed into an upcurrent-separator or jig or similar device, which in the case of the upcurrent-separator 80 separates the metalliferous granules from the gangue by allowing them to fall to the bottom of the vessel and to be carried away by a downward stream, while the particles of gangue are carried away by an upward stream. 85

The accompanying drawing is a diagram illustrating in sectional view one means of carrying out the process according to this invention.

A series of connected mixing vessels A' A<sup>2</sup> 90 A<sup>3</sup> A<sup>4</sup> A<sup>5</sup> A<sup>6</sup> are provided with stirrers B, rotated from driving-shafts B'. Crushed ore from a hopper C and circuit-water from a tank D are introduced into the first vessels A', and oil or emulsion is fed from a tank E, 95 through pipes E' E<sup>2</sup> E<sup>3</sup>, to the various vessels. The mixture is vigorously agitated to break up and emulsify the oil and to bring about in-

timate contact of the divided oil with the metalliferous mineral particles and of the oiled particles with each other. An alkaline emulsifying agent, such as soap, is introduced 5 into one or more of the vessels from a tank F, having discharge-pipes F<sup>3</sup> F<sup>4</sup> F<sup>5</sup> F<sup>6</sup>. It is found under these conditions that the metalliferous mineral particles abstract the oil and become coated with a thin oily film which is in- 10 sufficient to materially lessen their specific gravity and that under agitation such slightly-oiled particles adhere, nucleate, and agglomerate into small more or less rounded masses or granules disseminated throughout the mass 15 of gangue, which remains free and practically devoid of oil. After agitation to a certain extent (in four vessels, as illustrated, for example) the mixture is passed into an upcurrent-classifier G, which is supplied with a 20 stream of circuit-water from a tank H through a pipe H'. As the granules remain specifically heavier than the gangue or can by suitably adjusting the amount of oil and the agitation be obtained of a size larger than that 25 of the gangue particles, the granules, with a certain amount of heavy sands, sink to the bottom and are discharged through a pipe G' into vessel A<sup>5</sup>, while the lighter sands are carried away by the upward current and dis- 30 charged through outlet G<sup>2</sup> to a light-sands tank J, from which the circuit-water may be returned by a pump J' to the feed-tank D for reuse. In order to separate the granules from the heavy sands, the mixture is subjected to 35 further agitation in the vessels A<sup>5</sup> A<sup>6</sup> and is then passed into a second classifier K, from which the granules are removed at the bottom by the pipe K' into the metalliferous-mineral tank L, while the heavy sands are discharged 40 from the upper pipe K<sup>2</sup> into a heavy-sands tank M. The circuit-water from the tanks L and M is returned by a pump N' to the feed-water tank H. This apparatus is illustrated only as one convenient method of carrying 45 out this invention, and it is to be understood that its nature and arrangement can be considerably varied.

The water throughout the circuit is alkaline and contains a suitable proportion of soap or 50 other emulsifying agent. The agitation vessels may be separate, with arrangements for charging and discharging, the charging with pulp and the addition of oil or emulsified oil and the agitation and discharge successively 55 in the series of vessels being so timed that the output of treated ore is kept continuous and constant. The classifiers used may be jigs, shaking-tables, or the like or sizing apparatus whereby the comparatively larger mineral 60 granules may be separated from the finer gangue, and one or more classifiers may be employed.

The proportion of oil used depends upon its viscosity, the fineness of the ore, and other 65 factors, and the consistency and size of the

mineral granules desired. The more oil used the larger, softer, and less numerous the granules. With, say, ten per cent. of oil to the weight of metalliferous mineral a few pasty masses of oil agglomerated metalliferous mineral matter will generally result. Oil in excess of this may cause all the granules to coalesce into one soft mass. Usually an amount of oil varying from four per cent. to six per cent. of the weight of metalliferous mineral matter 70 present in the ore yields granules of suitable size, consistency, and specific gravity for ready separation from the gangue in the upcurrent or other apparatus used for classification. 75

The amount of emulsifying agent, if used to 80 form the oil-emulsion, depends upon the viscosity and nature of the oil. When soap is employed, an amount varying from three per cent. to five per cent. of the weight of oil usually suffices, this being dissolved in, say, ten times 85 its weight of water. For emulsification a low alkalinity of the emulsifying agent is generally best.

The oil used may be animal, vegetable, or mineral oil, or mixtures of these, or such 90 coal or wood tar products or other substances which exercise, like oils, a preferential physical affinity for metallic mineral matter as distinguished from gangue.

The emulsifying agent may be any substance 95 capable of holding the oil in a fine state of division in suspension in water without acting on the mineral matter or preventing the action of the oil—for example, soap, alkaline cresylates, or other substances solutions of which 100 in water froth on agitation. The emulsifying agent appears to have a decided effect in bringing about the granulation as described. In some cases, as with wood-tar and some coal-tar products, these when agitated in weak 105 alkaline solutions provide their own emulsifying agents, soluble resinate, cresylates, &c., being thereby formed, which emulsify the bulk of the tar or product.

Emulsification in some cases, as with the 110 heavier residuum oils or tars, may be assisted by first mixing therewith a small amount of fatty oil or fatty acid. Preferably one emulsifying agent is employed throughout the process.

In order to recover the oil from the granules after their separation from the gangue, they may be agitated with the emulsifying agent in a stronger or more active condition or proportion than was used in the emulsification of the oils initially, and the action of this emulsifying agent in stripping the oil from the metalliferous mineral particles may be aided by attrition. The strengthening of the emulsifying agent may be effected by increasing the proportion of the agent or of the alkaline base in solution, or both, the percentage strength of the solution needed depending upon the oil used and the nature of the metalliferous mineral matter with which it is 115 120 125 130

associated. Usually if oleic soap is employed and caustic potash amounts varying from one-quarter of one per cent. to three per cent. or four per cent. of one or the other in solution suffices, the less readily emulsified oils, as the residuum oils, requiring the larger amounts. The removed oil is obtained as a dilute emulsion, which on standing some time separates. The "cream" or concentrated emulsion may then be used for making fresh emulsion for treating fresh ore. To hasten this separation of cream, mechanical devices may be employed.

Generally with wet crushed ore removal of the bulk of the water for reuse in the mill is necessary. In such case the pulp is settled and the wet ore only fed into the agitators, emulsifying agent of suitable strength being added to thin them. The circuit of such liquids can thus be kept distinct from that of the mill-water, suitable arrangements being made for settling the mineral-depleted sands and slime and for addition of emulsifying agent and fresh water as required from time to time.

In certain cases, as where but little mineral is present in the ore, to increase the nucleating or granulating factor pulverized mineral matter obtained in a previous operation or other matter having an affinity for oil from a different source may be introduced into the ore, or a portion of already granulated and separated mineral matter may be returned to maintain the necessary amount of mineral in the ore under treatment.

In carrying out the process the ore may be roughly sized into two or more parts, which are then treated separately. With certain ores it may be preferable to use in some stages of the process a rolling form of agitation, as in cylinders or barrels, to obtain good granulation of the mineral.

It is preferable to use circuit-waters of varying degree of alkalinity, according to the nature of the mineral being treated, provided always that about one-half of one per cent. of soap or other emulsifying agent is present.

It is found advisable to keep the amount of free alkali low in proportion to the free soap present when such is the emulsifying agent used. Thus in one example 0.25 per cent. of free soap with 0.025 per cent. of free alkali was sufficient to keep calcite free from oil, 0.3 per cent. free soap and 0.03 per cent. free alkali kept quartz free from oil, while rather stronger solutions—as, for instance, 0.5 per cent. free soap and 0.05 per cent. free alkali—prevented garnet from becoming oil-coated. These figures refer to cases where a light oil was used—namely, paraffin. When the free soap was increased to about one per cent. or when the free alkali was increased to about one-fourth of one per cent., difficulty was found in agglomerating certain metalliferous

substances, such as rosin-blende and iron or copper pyrites. Care must therefore be taken that neither the soap nor the alkali is in excess of that required for preventing agglomeration of the gangue.

I am aware that the selective action of oils and the like on metallic matter has been made the basis of previous processes for separating the metalliferous constituents of ores from gangue. For example, oil has been used to float off metalliferous mineral from ore-pulp, and its use has also been proposed to form a pasty mass of crushed ore from which the gangue could afterward be washed out by means of water, and I do not claim the employment of oil in any such manner.

What I claim as my invention, and desire to secure by Letters Patent, is—

1. The herein-described process of separating metalliferous matter from gangue, which consists in agitating a mixture of powdered ore and water with oil in emulsion in water containing an alkaline emulsifying agent, so as to agglomerate the oil-coated particles into granules, and subjecting the mixture to classification to remove the small non-coated particles from the granules.

2. The herein-described process of separating metalliferous matter from gangue, which consists in agitating a mixture of powdered ore and water with oil in emulsion in water containing an alkaline emulsifying agent, so as to agglomerate the oil-coated particles into granules, and subjecting the mixture to up-current classification to remove the small non-coated particles from the granules.

3. The herein-described process of separating metalliferous matter from gangue, which consists in forming granules by agitating a mixture of powdered ore and water with oil in emulsion in water containing an alkaline emulsifying agent, separating out the light sands, and thereafter further agitating the pulp to increase the size of the granules and separating out the heavy sands from the granules.

4. The herein-described process of separating metalliferous matter from gangue, which consists in agitating a mixture of powdered ore and water with oil in emulsion in water containing an alkaline emulsifying agent, adding particles of material having an affinity for oil to assist in the formation of granules of oil-coated particles, and subjecting the mixture to classification to remove the small non-coated particles from the granules.

In testimony whereof I have signed my name to this specification in the presence of two subscribing witnesses.

ARTHUR EDWARD CATTERMOLE.

Witnesses:

CHRISTOPHER BARNETT,  
WALTER J. SKERTEN.